

# UNITED STATES PATENT OFFICE.

RASMUS BECK, OF DÜREN, GERMANY, ASSIGNOR TO THE FIRM OF DÜRENER METALLWERKE AKTIEN-GESELLSCHAFT, OF DÜREN, GERMANY.

## GERMAN-SILVER-ALLOY PRODUCTS AND MANUFACTURE OF SAME.

1,227,569.

Specification of Letters Patent.

Patented May 29, 1917.

No Drawing.

Application filed June 27, 1914. Serial No. 847,694.

To all whom it may concern:

Be it known that I, RASMUS BECK, a citizen of the German Empire, residing at Düren, Germany, have invented certain new and useful Improvements in German-Silver-Alloy Products and Manufacture of Same, of which the following is a specification.

This invention relates to rolled, drawn, extruded, stamped or forged products of German silver. For this purpose a German silver alloy, that is to say a zinc-copper-nickel alloy, of special composition is used which is distinguished from other German silver alloys by its property of allowing working at red heat, and from such alloy the products are manufactured by working the metal at red heat at least during a large part of the working processes.

The alloy composition which is suited for the purpose is a composition comprising besides 40 to 50% of zinc about 10% of nickel whereas the rest is formed entirely or mostly from copper.

It is not necessary to adhere strictly to the above named proportion of nickel. The increase or decrease in the nickel percentage shall, however, not be more than 5%, that is the alloy shall contain between 5% and 15% nickel, this being a condition for obtaining alloys which are at the same time workable while hot and of silver-white color, especially if part of the nickel is replaced by other compounds of same coloring action. By going below the lower limit, the alloy loses its silver-white color and besides becomes brittle; by going above the higher limit the alloy loses to a very great extent its property of being workable at red heat.

However, nickel may be replaced in small parts by other metals which, like nickel, may be designated as white metals, such as cobalt, manganese, iron, aluminium, tin, magnesium and lead according to the qualities required from the manufactured products, the total contents in copper, nickel, and such other metals again amounting to 50-60%.

The economic importance of the invention resides in the cheapness of the metal used as well as in the cheapness of the working process. The cheapness of the metal results from the low percentage of nickel with a low percentage of copper, and the cheapness of the working process results

from the working being done at red heat. Moreover, the invention allows of producing objects of German silver which can only be worked warm, such as extruded shapes by the extrusion process and stampings and forgings. Other products in German silver alloys, such as sheets, strips, wires, and tubes which heretofore were only worked cold from alloys high in copper and nickel are cheapened on account of their being manufactured warm during a large part of the processes.

One of the characteristics of the new German silver alloy products is their high tensile strength; for instance annealed extruded rods of an alloy containing

46 Cu-8Ni-2Mn-44Zn

having a silver-white color and being very readily workable proved to possess a tensile strength of 36 kilograms per square millimeter or 22.84 tons per square inch at the elastic limit, 70 kilograms per square millimeter or 44.42 tons per square inch at the breaking stress limit with an elongation of 20%.

The high tensile strength characteristics allow the use of the new alloy for such construction purposes for which a high tensile strength is required.

What I claim is:

1. The method of forming articles from a German silver alloy consisting of 40-50% of zinc, 5-15% of white metal in which nickel largely preponderates and the residue of copper, which consists in heating the alloy to red heat and working it while hot into the desired shape.

2. The method of forming articles from a German silver alloy consisting of from 40-50 per cent zinc, approximately 10 per cent of nickel, and the residue of copper, which consists in heating the alloy to about red heat and working it while hot into the desired shape.

3. Rolled, drawn, extruded, stamped, forged, and similar products of German silver alloy containing 40-50 per cent. of zinc, and 5 to 15 per cent. of other white coloring metals, the residue consisting mainly of copper.

4. Rolled, drawn, extruded, stamped, forged and similar products of German silver alloy containing 40-50 per cent. of zinc and 5 to 15 per cent. of other white coloring

85

90

100

105

110

metals in which nickel largely predominates, the residue consisting mainly of copper.

5. Rolled, drawn, extruded, stamped, forged, and similar products of German silver alloy containing 40-50 per cent. of zinc, and 5 to 15 per cent. of nickel and at least one of the following white coloring metals: cobalt, manganese, iron, aluminum, tin, magnesium, and lead, the nickel largely pre-

dominating among said white coloring metals, the residue consisting mainly of copper.

In testimony whereof I affix my signature in presence of two witnesses,

RASMUS BECK.

Witnesses:

PAUL DREES,

HENRY QUADFLIEG.